

No. 616,276.

Patented Dec. 20, 1898.

O. M. THOWLESS.

ILLUMINANT FOR INCANDESCENT ELECTRIC LAMPS AND PROCESS OF MAKING.

(Application filed Jan. 31, 1896.)

(No Model.)

*Fig. 1. Thorium Oxide*



*Fig. 2.*



WITNESSES:

*Ethan D. Dodes*  
*Hubert C. Tener*

INVENTOR

*Orlando M. Thowless*

BY  
*Charles A. Tracy*  
ATTORNEY

# UNITED STATES PATENT OFFICE.

ORLANDO M. THOWLESS, OF NEWARK, NEW JERSEY.

## ILLUMINANT FOR INCANDESCENT ELECTRIC LAMPS AND PROCESS OF MAKING.

SPECIFICATION forming part of Letters Patent No. 616,276, dated December 20, 1898.

Application filed January 31, 1896. Serial No. 577,513. (No model.)

*To all whom it may concern:*

Be it known that I, ORLANDO M. THOWLESS, a subject of the Queen of Great Britain, residing at Newark, county of Essex, and State 5 of New Jersey, have invented certain new and useful Improvements in Illuminants for Incandescent Electric Lamps and in Processes of Making the Same, of which the following is a specification.

10 My invention relates to the construction of the illuminating portion of an incandescent electric lamp.

The object of my invention is to provide an illuminant which will yield a greater amount 15 of light than is ordinarily obtained from an incandescent filament of the usual construction by the consumption of a given amount of electrical energy.

15 My invention comprises a new process or method of operation and a new product produced thereby. This new product may be generally described as an illuminant for incandescent electric lamps consisting of a filament inclosed within a sheath or covering 25 of material possessing the property of illuminating readily by the action of an electric current.

The material may be one of the class having the general characteristics of an 30 oxid of thorium, zirconium, yttrium, or lan-

thanum or some other metallic oxides of the 35 same general characteristics, and the new process consists of the novel method of obtaining the product, which is accomplished by preparing on the filament a combustible 40 material—such, for instance, as cotton—im- pregnated with the salts of one or more metals, then destroying the combustible material and reducing the metallic salts to their corresponding metallic oxides, thereby forming 45 on the filament a sheath or cover of metallic oxid. This method and its modifications are hereinafter more fully described.

It has heretofore been suggested that a carbon incandescent conductor be coated with 50 some refractory material; but no practicable method has been ascertained for so doing. By my invention I am enabled to secure a coating which illuminates readily, and find the same to be durable and efficient.

55 A method of applying the coating which I have found successful consists in threading a carbonized filament of the usual well-known

character through a sheathing or tube of woven fibrous material—such, for instance, as cotton. This is then impregnated with a 55 salt, in solution, of thorium or zirconium, yttrium or lanthanum, or some other suitable salt the oxid of which possesses in a high degree the property of illuminating readily and is capable of withstanding an intense 60 heat. The nitrate of thorium, for example, gives excellent results. The strength of the solution may be varied as required for the purpose of giving to the completed filament a greater or less amount of coating. The fila- 65 ment, with its coating, is then dried, and the fibrous structural coating or tube is then removed by heat—as, for instance, by placing it in a furnace or oven, where sufficient heat may be applied to destroy the cotton or other 70 fiber and reduce the salt to an oxid, thus leaving a coating of the oxid of the metal in close proximity to the filament. After the filament has thus been prepared it is then in condition to be placed in the usual form of vacuum- 75 chamber or lamp-globe and exhausted in the usual well-known manner.

Instead of threading the filament through the covering of fibrous material the latter may be woven upon or otherwise applied to 80 the filament.

The sheathing, tube, or covering may be soaked in the solution of the metallic salt before it is applied to the filament, and, indeed, the cotton or other material of which the 85 cover is to be formed may be treated with metallic salts before it is woven or otherwise shaped.

A lamp thus made is found to be durable 90 and efficient, and the light-giving properties of the filament are materially enhanced by the presence of the coating. The coating adheres more or less closely to the surface of the filament, and this intimate relation of the metallic oxid with the filament secures stability for the entire structure. This method of applying the coating permits the necessary 95 expansion and contraction of the filament without causing the coating to be broken.

Various different salts of the metals may 100 be applied in practice.

A modification in the process of applying the coating to the filament consists in first impregnating one coating in the manner al-

ready described and afterward forming one or more additional coatings of either the same or of different oxids in essentially the same manner.

- 5 Another modification consists in impregnating the coverings of the filament with salts of two or more different metals before the preliminary heating, and this may be done either by soaking the filament and its fibrous 10 covering in the salts of the metals successively or in a mixture of two or more of such salts simultaneously, or after one such coating has been so treated another fibrous tube or covering may be superposed and the treatment 15 repeated. The fibrous covering is then destroyed and the salts reduced to their respective oxids.

Heretofore filaments for incandescent electric lamps have usually been made of carbon. 20 My invention is applicable not only to such filaments, but also to filaments of metal, the process of applying the coating being essentially the same as that above described.

In the accompanying drawings, Figure 1 is 25 an illustration of a filament covered with a coating of combustible material, and Fig. 2 is an illustration of a completed lamp.

Referring to the figures, *a* represents a filament of any suitable character, and *b* represents the covering of cotton or other combustible material. A suitable inclosing bulb 30 is represented at *C*, Fig. 2, and the parts *d d* represent leading-in wires for supporting the completed illuminant *e*.

35 I claim as my invention—

1. The hereinbefore-described method of applying a coating of refractory material to a filament for incandescent electric lamps, which consists in first applying a covering of 40 readily-combustible material to the surface of the filament, impregnating the same with a salt of thorium or other metal, and removing the covering of combustible material by heat or decomposition.

45 2. The hereinbefore-described method of preparing incandescent-electric-lamp fila-

ments which consists in incasing the length of the filament in a continuous woven sheathing, impregnating the same with a metallic salt, and removing the coating of woven material by heat, and reducing the metallic salt to a metallic oxid, substantially as described. 50

3. The hereinbefore-described method of preparing incandescent conductors for electric lamps which consists in incasing a filament in a covering of combustible material impregnated with a metallic salt, and removing such combustible material by heat or decomposition and reducing the metallic salt to a metallic oxid. 55

4. The hereinbefore-described method of preparing conductors for incandescent electric lamps, which consists in incasing a filament in a covering of combustible material impregnated with two or more metallic salts, 60 destroying such combustible material, and reducing the salts of the metals to the corresponding metallic oxids.

5. The method of preparing conductors for incandescent electric lamps which consists in 70 incasing a filament in a covering of combustible material, impregnated with a metallic salt, subjecting the same to a bath of one or more other metallic salts, and then destroying the covering of combustible material. 75

6. An illuminant for incandescent electric lamps consisting of a carbon filament and a surrounding sheath or covering of oxid or other compound of thorium.

7. An illuminant for incandescent electric 80 lamps consisting of a filament, a surrounding sheath or covering of oxid or other compound of thorium, or its equivalent, and an exhausted bulb containing the same.

In testimony whereof I have hereunto subscribed my name this 24th day of January, A. D. 1896.

ORLANDO M. THOWLESS.

Witnesses:

H. A. CROOKS,  
W. D. UPTEGRAFF.